

## UNITED STATES PATENT OFFICE.

GEORGE HOLLAND ELLIS, OF SPONDON, NEAR DERBY, ENGLAND, ASSIGNOR TO CELANESE CORPORATION OF AMERICA, A CORPORATION OF DELAWARE.

## TREATMENT OF CELLULOSE ACETATE.

No Drawing. Application filed August 15, 1925, Serial No. 50,525, and in Great Britain September 19, 1924.

This invention relates to dyeing, printing or stencilling (all hereinafter in the claims included in the term dyeing) of yarns, threads, filaments, fabrics, films or other products 5 made of or containing cellulose acetate, all hereinafter in the claims included in the term materials comprising cellulose acetate.

In my U. S. Patent No. 1,618,413, there is described processes for dyeing, printing or 10 stencilling the goods of or containing cellulose acetate by colouring matters or organic compounds having affinity for cellulose acetate or capable of colouring the same, but which are insoluble or practically insoluble 15 in water or are of relatively low solubility in water, said colouring matters or organic compounds being employed in the form of soluble or more soluble modifications obtained by treating them prior to addition to 20 the dyebaths or preparations for printing and the like, with bodies having oily or fatty characteristics, namely higher fatty acids or sulphated or other derivatives thereof containing salt-forming groups, e. g. the sulpho 25 group, carboxyl group or salts of such acids or derivatives.

According to the present invention I employ for the dyeing, printing or stencilling of cellulose acetate or goods containing the 30 same any insoluble or relatively insoluble colouring matters or compounds having affinity for cellulose acetate or capable of dyeing the same all of which are hereinafter in the claims included in the expression "relatively 35 water-insoluble organic compounds capable of coloring cellulose acetate", in the form of soluble or more soluble modifications prepared by pretreatment with solubilizing agents consisting of or comprising one or 40 more bodies being Twitchell reagents, which expression includes sulphoaromatic fatty acids, such as sulphobenzene stearic acid, sulphophenol stearic acid, or sulphonaphthalene stearic acid, and salts of sulphoaromatic 45 fatty acids.

As before stated any insoluble or relatively insoluble colouring matter or compound having affinity for cellulose acetate or capable of coloring the same may be used for the present invention. Thus for example I may employ insoluble or relatively insoluble colouring matters or compounds more particularly specified in the previous U. S. application

Serial No. 664,780, Patent No. 1,618,413, for instance, non-sulphonated or other insoluble 55 or relatively insoluble derivatives of the "azo" class, simple amino bases, unreduced indophenols (aryl or substituted aryl benzo-naphtho quinonemonoimides) or insoluble or relatively insoluble colouring matters of the following classes: polyphenyl methane, oxazine, azine, thiazine, unreduced indigoid or basic derivatives of the anthraquinone series.

Or, for example, I may employ insoluble or relatively insoluble pyrazolone derivatives e. 65 g. unsulphonated azo derivatives of pyrazolone compounds such as are specified in the previous U. S. application Serial No. 737,903, filed 15 September, 1924 Patent No. 1,600,277.

Or, for example, I may employ the insoluble 70 or relatively insoluble colouring matters specified in the previous U. S. application Serial No. 740,413, filed 27 September, 1924, Patent No. 1,641,965, i. e. vat dyestuffs of the anthraquinone series in the unreduced state, 75 for example indanthrene, cibanone, algol, helindone or other vat dyestuffs of the anthraquinone series in the unreduced state.

Or, for example, I may employ insoluble 80 or relatively insoluble nitro derivatives of diarylamine such as are specified in U. S. application S. No. 6,460, filed 2 February, 1925 Patent No. 1,618,415.

It is to be understood that any other insoluble or relatively insoluble colouring matter or 85 compound having affinity for cellulose acetate or capable of colouring the same may be used for the process of the present invention.

The insoluble or relatively insoluble colouring matters or compounds for use in the present invention will usually contain no strongly 90 acidic groups such as the sulpho group and when basic colouring matters or compounds are employed they are always used in form of the base and not in the form of salts such 95 as the hydrochloride or other such salt.

The solubilization of the aforesaid insoluble or relatively insoluble colouring matters or compounds may be effected by mixing or 100 grinding them with one or more of the solubilizing agents of the present invention, in presence or absence of water and heating if necessary, the solubilized modifications being filtered if desired before addition to the dyebaths or other preparations for dyeing or 105 otherwise colouring the goods containing

cellulose acetate. The dyeing or otherwise colouring of the goods may be effected in the usual manner.

If the colouring matter or compound applied according to the process of the present invention contains diazotizable primary amino groups, it may be diazotized and developed on the material in the usual manner to form a further dyestuff or dyestuffs.

10 When dyeings or colourings are to be produced by the azoic process (i. e. wherein the actual dyestuffs are produced on the material by coupling of simple amino bases with developers on the material) the insoluble or relatively insoluble component (whether base or developer) may be solubilized with the agents of the present invention and the dyeing or developing conducted as usual.

With reference to dyeing or coloring by means of the azoic process, wherein the actual dyestuffs are produced on the cellulose acetate fibre or material by the coupling of simple amino bases with developers, it is understood that the expression "organic compound capable of coloring cellulose acetate" employed in the claims applies to said bases or developers in the sense that they are capable of coloring the cellulose acetate by such production of a dye thereon, whether or not the bases or developers themselves color cellulose acetate.

Other colouring matters which are not deleteriously affected by the solubilizing agents of the present invention may, if desired, be dyed on the material together with the colouring matters or compounds of the character before indicated.

Mixed goods may be dyed or otherwise coloured in uniform or contrasting effects with or without employment of other dyestuffs or components according to the character of the non-acetate portion of the goods, said other dyestuffs or components being applied if desired before or after the application of the hereinbefore specified insoluble or relatively insoluble dyestuffs or compounds or when not deleteriously affected thereby they may be applied in conjunction therewith.

50 The solubilizing agents employed according to the present invention as hereinbefore referred to, may be prepared in any known or suitable way. The following examples A. and B. may conveniently be given to illustrate methods by which sulpho aromatic fatty acid solubilizing agents such as referred to may be prepared, it being of course understood that I in no way limit myself to the use of solubilizing agents so prepared and that I may use any other solubilizing agents hereinbefore indicated.

A. 25 kilogs. of naphthalene are mixed with 25 kilogs. of oleic acid by warming to 80° C. The mass is then cooled quickly and the resultant paste is added slowly to 100

kilogs. of 20% oleum with vigorous agitation, the temperature being kept below 40° C. When the addition is complete the temperature is raised very gradually to 100° C. at which it is maintained for 3 hours. Care is needed during this heating to prevent a frothing. After cooling, the mixture is poured into 250 litres of water and treated with 50 kilogs. of common salt. The whole is allowed to separate, when the top aqueous layer is decanted off leaving an oily product which is washed several times with 20% brine. The product is then suitable for use for solubilization or dispersion of colouring matters or dyestuffs in accordance with the present invention. Where desired it may be neutralized or made alkaline with requisite quantities of caustic soda.

75 B. The process described in A. is repeated exactly but substituting the naphthalene by an equal weight of benzene. Owing to the lower boiling point of the latter the operation of heating is done under reflux, working up on the same lines as in A.

80 The following examples will serve to illustrate how the invention may be carried out, it being understood that they are in no way limitative and may be varied widely.

#### Example 1.

To dye a brilliant orange shade on 100 kilogs. of cellulose acetate yarns in the form of hanks, 4 kilogs. of paranitro-benzene-azo-diphenylamine 25% aqueous paste are finely ground and 3-4 kilogs. of the sulpho-aromatic fatty acid product prepared according to A. are added, the whole being well stirred. The mixture is heated until the maximum degree of dispersion is achieved and then diluted with boiling water and passed through a sieve into a suitable dyeing machine or vat containing water acidified with 2 litres of formic acid 80%. The goods are entered and the temperature raised according to the common methods of dyeing until the shade is achieved.

#### Example 2.

To dye a shade of reddish blue on 25 kilogs. of cellulose acetate woven fabric, 2 kilogs. of 25% aqueous paste of dimethyl-para-amino-phenyl-1:4-naphthoquinone-monoimide are mixed with 2 kilogs. of a sulphoaromatic fatty acid in the form of its sodium salt prepared according to A. above, and the whole is heated to obtain good dispersion. The resultant mass is diluted with boiling water and added through a sieve to a suitable machine such as a dye jigger containing soft water. The goods are entered and passed through repeatedly in the manner common with this machine. The goods are then rinsed, dried and finished as is requisite.

#### Example 3.

To dye a brilliant scarlet red shade by the

azoic process on 100 kilogs. of cellulose acetate fabric, 1 kilog. of finely ground amido-azobenzene base is treated with 4 kilogs. of a sulphoaromatic fatty acid preparation, made according to A. The mass is stirred and heated until the maximum dispersion is obtained when it is well diluted with boiling water and the preparation added through a sieve to a suitable dyeing machine for example of the winch or reel type containing a sufficiency of water acidulated with 4 litres of acetic acid 40%. The temperature is raised until the bath is as well exhausted as required. The goods are rinsed and then the base diazotized with sodium nitrite and hydrochloric acid and again rinsed and developed with sodium betanaphtholate according to procedures well known in the art.

*Example 4.*

To dye a very fast to light shade of sky blue on 100 kilogs. of cellulose acetate woven fabric, 10 kilogs. of 1-monomethyl-amino-4-paratolylamino-anthraquinone 25% aqueous paste are treated with 10 kilogs. of a sulphoaromatic acid preparation made as described in B. above. The mass, after being well mixed is heated to obtain the maximum degree of dispersion possible, and then diluted with boiling water and added to water contained in the beck of a jig type of machine. The rolled up goods are entered in the usual manner when dyeing on this type of machine and passed through continuously with raising of temperature until the desired shade has been obtained, when rinsing and any after-treatment or finishing in common practice may follow.

*Example 5.*

To dye a brilliant bluish green on 100 kilogs. of cellulose acetate yarns in the form of hanks, 2 kilogs. of tetramethyldiparaminotriphenylcarbinol (malachite green base) are finely ground and mixed with 8 kilogs. of sulpho aromatic fatty acid prepared according to B. above. The mass is heated to obtain the maximum degree of dispersion and then diluted with boiling water and added through a sieve to a dye-bath containing a sufficiency of water, say 3,000 litres. The goods are entered at a temperature of 45° C. and worked in a suitable manner, the temperature being raised until the maximum degree of exhaustion is obtained. A warm rinse with water acidified with acetic or formic acid preferably follows, afterwards further rinsing, drying and finishing as desired.

*Example 6.*

To dye a brilliant shade of yellow on the cellulose acetate and a bright blue shade on the wool components respectively in 200 kilogs. of mixed knitted fabric containing

equal proportions of the two fibres, 6 lbs. of a 25% aqueous paste of 4-chlor-2-nitrophenyl-4'tolylamine are well ground and treated with 6 kilogs. of sulphoaromatic fatty acid prepared according to A and the mass heated to obtain maximum dispersion. Boiling water is then added and the hot liquid then passed through a sieve into a suitable dyeing machine such as winch or reel type commonly employed containing 5,000 litres of water acidified with 4 kilogs. of formic acid 90%. To the above dye bath is then added a solution of 2 kilogs. of the diamino-anthrarufin-disulphonic acid dyestuff known as Alizarin Delphinol B. in a sufficiency of water. The goods after suitable scouring are entered and dyed with raising of temperature to a maximum preferably not above 80° C. common salt being added as desired, according to the depth of shade. When this has been achieved on the two components the goods are washed, dried and finished as requisite.

*Example 7.*

To dye a shade of lemon yellow on 25 kilogs. of woven fabric made from cellulose acetate yarns 125 grams of benzene-azophenylmethylpyrazolone are finely ground with 375 cc. of water and 500 grams of sulphoaromatic fatty acid preparation according to B. above is added and whole stirred and heated to obtain maximum dispersion. It is then diluted with boiling water and passed through a sieve to the dyebath which may take the form of the jig type of machine. This dyebath should contain a sufficiency of water acidified with 250 grams of acetic acid 100%. The goods are worked through the bath, raising the temperature until the requisite shade is achieved when the usual rinsing and finishing processes as desired may follow.

*Example 8.*

To print a shade of Tangerine on cellulose acetate woven fabric, the paranitrobenzene-azodiphenylamine preparation obtained according to Example 1, above is diluted, instead of with plain water, with an aqueous thickening of gum arabic and corn starch of suitable consistency for roller machine printing. The paste is acidified so as to contain 5 cc. per liter of 100% formic acid and is well boiled to give the highest degree of dispersion possible. After cooling it is applied in the usual manner in printing. The print is dried, aged for 15 min. in dry steam and is then well washed, dried and finished as desired.

What I claim and desire to secure by Letters Patent is:

1. A process for the dyeing of materials comprising cellulose acetate which comprises treating said materials with relatively water insoluble organic compounds capable of coloring cellulose acetate, said organic com-

pounds being employed in the form of solubilized modifications obtained by pretreating them with a solubilizing agent comprising a Twitchell reagent.

5. 2. A process for the dyeing of materials comprising cellulose acetate which comprises treating said materials with relatively water insoluble organic compounds capable of coloring cellulose acetate, said organic compounds being employed in the form of solubilized modifications obtained by pretreating them with a solubilizing agent comprising a sulphonaphthalene stearic acid body.

10. 3. A process for the dyeing of materials comprising cellulose acetate which comprises treating said materials with relatively water insoluble organic compounds capable of coloring cellulose acetate, said organic compounds being employed in the form of solubilized modifications obtained by pretreating them with a solubilizing agent comprising a salt of sulphonaphthalene stearic acid.

15. 4. A process for the dyeing of materials comprising cellulose acetate which comprises treating said materials with relatively water insoluble organic compounds capable of coloring cellulose acetate, said organic compounds being employed in the form of solubilized modifications obtained by pretreating them with a solubilizing agent comprising sodium salt of sulphonaphthalene stearic acid.

20. 5. A process for the dyeing of materials comprising cellulose acetate which comprises treating said materials with relatively water insoluble organic compounds of the azo class capable of coloring cellulose acetate, said organic compounds being employed in the form of solubilized modifications obtained by pretreating them with a solubilizing agent comprising a Twitchell reagent.

25. 6. A process for the dyeing of materials comprising cellulose acetate which comprises treating said materials with relatively water insoluble organic compounds of the azo class capable of coloring cellulose acetate, said organic compounds being employed in the form of solubilized modifications obtained by pretreating them with a solubilizing agent comprising a sulphonaphthalene stearic acid body.

30. 7. A process for the dyeing of materials comprising cellulose acetate which comprises treating said materials with relatively water insoluble organic compounds of the azo class capable of coloring cellulose acetate, said organic compounds being employed in the form of solubilized modifications obtained by pretreating them with a solubilizing agent comprising a salt of sulphonaphthalene stearic acid.

35. 8. A process for the dyeing of materials comprising cellulose acetate which comprises treating said materials with relatively water insoluble organic compounds of the azo class

capable of coloring cellulose acetate, said organic compounds being employed in the form of solubilized modifications obtained by pretreating them with a solubilizing agent comprising sodium salt of sulphonaphthalene stearic acid.

9. A process for the dyeing of materials comprising cellulose acetate which comprises treating said materials with paranitrobenzene azo diphenylamine in the form of a solubilized modification obtained by pretreating it with a solubilizing agent comprising a Twitchell reagent.

10. A process for the dyeing of materials comprising cellulose acetate which comprises treating said materials with paranitrobenzene azo diphenylamine in the form of a solubilized modification obtained by pretreating it with a solubilizing agent comprising a sulphonaphthalene stearic acid body.

15. 11. A process for the dyeing of materials comprising cellulose acetate which comprises treating said materials with paranitrobenzene azo diphenylamine in the form of a solubilized modification obtained by pretreating it with a solubilizing agent comprising a salt of sulphonaphthalene stearic acid.

20. 12. A process for the dyeing of materials comprising cellulose acetate which comprises treating said materials with paranitrobenzene azo diphenylamine in the form of a solubilized modification obtained by pretreating it with a solubilizing agent comprising sodium salt of sulphonaphthalene stearic acid.

25. 13. A process for the dyeing of mixed materials comprising cellulose acetate and other fibre which comprises treating said materials with relatively water insoluble organic compounds capable of coloring cellulose acetate, said organic compounds being employed in the form of solubilized modifications obtained by pretreating them with a solubilizing agent comprising a Twitchell reagent.

30. 14. A process for the dyeing of mixed materials comprising cellulose acetate and other fibre which comprises treating said materials with relatively water insoluble organic compounds capable of coloring cellulose acetate, said organic compounds being employed in the form of solubilized modifications obtained by pretreating them with a solubilizing agent comprising a sulphonaphthalene stearic acid body.

35. 15. A process for the dyeing of mixed materials comprising cellulose acetate and other fibre which comprises treating said materials with relatively water insoluble organic compounds capable of coloring cellulose acetate, said organic compounds being employed in the form of solubilized modifications obtained by pretreating them with a solubilizing agent comprising a salt of sulphonaphthalene stearic acid.

40. 16. A process for the dyeing of mixed materials comprising cellulose acetate and other



- relatively water insoluble organic compounds capable of coloring cellulose acetate, said relatively water insoluble organic compounds being employed in the form of solubilized 5 modifications obtained by pretreating them with a solubilizing agent comprising sodium salt of sulphonaphthalene stearic acid.
29. A composition of matter applicable for the dyeing of cellulose acetate, comprising 10 a solubilized modification of a relatively water insoluble organic compound capable of coloring cellulose acetate, said solubilized modification comprising a Twitchell reagent as a solubilizing agent.
- 15 30. A composition of matter applicable for the dyeing of cellulose acetate comprising a
- solubilized modification of a relatively water insoluble organic compound capable of coloring cellulose acetate, said solubilized modification comprising a sulphonaphthalene stearic acid body as a solubilizing agent. 20
31. A composition of matter applicable for the dyeing of cellulose acetate, comprising a solubilized modification of a relatively water insoluble organic compound capable of coloring cellulose acetate, said solubilized modification comprising sodium salt of sulphonaphthalene stearic acid as a solubilizing agent. 25
- In testimony whereof I have hereunto sub- 30  
scribed my name.

GEORGE HOLLAND ELLIS.